

# UNITED STATES PATENT OFFICE.

WILLIAM JACOB KUHNS, OF BROOKLYN, NEW YORK.

## IMPROVEMENT IN NICKEL PLATING.

Specification forming part of Letters Patent No. 103,201, dated May 17, 1870.

I, WILLIAM JACOB KUHNS, of Brooklyn, county of Kings and State of New York, have invented a certain Improvement in the Process of Nickel Plating by the battery, of which the following is a specification:

The object of my invention is to secure a more perfect contact and adhesion of the nickel upon the surface of the article to be nickel plated; and my process is especially useful for nickel plating on iron and steel.

My improvement consists in causing a film of tin to lie between the surface of the article to be nickel plated and the film of nickel. The office of the tin is to serve as a bond of union between the substance of the article to be plated and the nickel. The surface-metal of the article has little affinity for the nickel, while both of these strongly adhere to tin.

The coating of tin is given to the article to

be plated in any of the known efficient methods—as, for example, by dipping in molten tin, by boiling, or by the battery.

After the coating of the article with tin, the nickel is deposited on the tinned surface by means of the galvanic battery in the ordinary manner.

I claim as my invention—

1. The use of a film of tin in the art of nickel plating, in the manner and for the purpose described.
2. The combination of films of tin and nickel, when the nickel has been deposited by a galvanic battery.

W. J. KUHNS.

Witnesses:

CHARLES A. SEELEY,  
J. H. HAVENS.